

3,000,953

## TETRANITRAMINES

Milton B. Frankel, Pasadena, Calif., assignor to Aerojet-General Corporation, Azusa, Calif., a corporation of Ohio

No Drawing. Filed June 13, 1957, Ser. No. 666,271  
16 Claims. (Cl. 260—583)

This invention relates to new compositions of matter and to the preparation thereof. More particularly, this invention relates to high energy tetranitramines of the following general formula:



wherein R is a hydrogen, alkyl or nitroalkyl radical and A is an alkylene radical.

The high energy tetranitramines of this invention are useful as high explosives and can be used in any conventional explosive missile, projectile, rocket, or the like, as the main explosive charge. An example of such a missile is disclosed in United States Patent No. 2,470,162, issued May 17, 1949. One way of using the high explosives of this invention in a device such as that disclosed in United States Patent No. 2,470,162, is to pack the crystalline explosive in powder form into the warhead of the missile. Alternatively, the crystals can be first pelletized and then packed. A charge thus prepared is sufficiently insensitive to withstand the shock entailed in the ejection of a shell from a gun barrel or from a rocket launching tube under the pressure developed from ignition of a propellant charge, and can be caused to explode on operation of an impact- or time-fuse mechanism firing a detonating explosive such as lead azide or mercury fulminate.

The high energy tetranitramines of my invention are prepared by reacting a dinitramine with nitric acid in accordance with the general reaction scheme set forth below:



wherein R and A are as defined above.

To more clearly illustrate my invention, the following example is presented. It should be understood that this example is presented merely as a means of illustration and is not intended to limit the scope of the invention to the particular conditions set forth therein.

*Example 1.—Preparation of 2,5,9,12-tetraaza-2,5,7,7,9,12-hexanitrotridecane*

A mixture of 200 ml. of 99% nitric acid, 200 ml. of concentrated sulfuric acid and 25 g. of 2,5,9,12-tetraaza-2,7,7,12-tetranitrotridecane was maintained within the temperature range of 50°—55° C. for thirty minutes and then cooled and poured on ice. The product was obtained as white solid, washed with water, and dried; 13.19 g. of a material having an M.P. of 94°—96° C. was obtained. The product, 2,5,9,12-tetraaza-2,5,7,7,9,12-hexanitrotridecane, was recrystallized from concentrated nitric acid and then from ethylene dichloride to produce a final material having an M.P. of 115°—117° C.

*Analysis.*—Calculated for  $\text{C}_9\text{H}_{18}\text{N}_{10}\text{O}_{12}$ : Percent C, 23.58; percent H, 3.96; percent N, 30.56. Found: Percent C, 21.65; percent H, 3.66; percent N, 28.92.

The reaction temperature is not critical in the practice of this invention, the only effect of temperature variation being a corresponding increase or decrease in reaction rate.

It is preferred to carry out the nitration reaction of the present invention in the presence of a dehydrating agent such as sulfuric acid. The dehydrating agent takes up the water of reaction thereby shifting the reaction equilibrium so as to increase the product yield. My invention is not limited to the use of sulfuric acid as a dehydrating agent. Other conventional dehydrating agents such as acetic anhydride, phosphoric acid, phosphoric anhydride, lower organic acid anhydrides such as butyric acid, propionic acid, etc., anhydrides, trifluoroacetic anhydride, or their equivalents can be used in the practice of my invention.

The dinitramines used as starting materials for the preparation of the high energy tetranitramines of this invention are obtained by condensing nitraza amines, such as 3-nitraza-1-butylamine, with 2,2-dinitro-1,3-propanediol, as more fully disclosed in my copending U.S. patent application Serial No. 666,275, filed concurrently with the present application. In condensing the nitraza amines with the 2,2-dinitro-1,3-propanediol, it is preferred to generate the nitraza amines from strong mineral acid salts thereof in situ, preferably by neutralizing the salts with inorganic basic salts of alkali or alkaline earth metals such as sodium hydroxide, lithium carbonate, calcium bicarbonate, etc., or with weak organic acid salts of alkali or alkaline earth metals such as potassium acetate, magnesium butyrate, etc.

The strong mineral acid salts of nitraza amines from which the free nitraza amines generated in situ, as described above, are prepared by reacting corresponding nitraza isocyanates, such as 3-nitraza-1-butyl isocyanate, with aqueous solutions of strong mineral acids, for example, hydrochloric acid, nitric acid, etc., as more fully described in my copending U.S. patent application Serial No. 666,273, filed concurrently with the present application.

It should be noted that the dinitramine starting materials of the present invention can be those which have been prepared from mixtures of nitraza amines as well as those prepared from individual nitraza amines. Thus, unsymmetrical dinitramines, such as those in which the two R's and/or the two A's as shown in the general formula are not identical can be nitrated by the method of my invention to form corresponding unsymmetrical tetranitramines.

It will be appreciated that a wide variety of tetranitramine compounds within the scope of my invention can be prepared by the method of this invention. For example, 3,7,11,15-tetraaza-3,9,9,15-tetranitroheptadecane; 2,2,4,9,9,14,16,16-octanitro-4,7,11,14-tetraazaheptadecane; and 2,2,4,9,9,15-hexanitro-4,7,11,15-tetraazaheptadecane can be nitrated to yield 3,7,9,9,11,15-hexanitro-3,7,11,15-tetraazaheptadecane; 2,2,4,7,9,9,11,14,16,16-decanitro-4,7,11,14-tetraazaheptadecane; and 2,2,4,7,9,9,11,15-octanitro-4,7,11,15-tetraazaheptadecane, respectively. Other members of this new series of compounds are prepared simply by reacting appropriate starting materials according to the teachings of this invention.

I claim:

1. As a composition of matter, a tetranitramine having the formula:



wherein R is a radical selected from the group consisting of hydrogen, lower alkyl and lower nitroalkyl radicals and A is a lower alkylene radical.

2. As a composition of matter, a tetranitramine having the formula:



wherein R is a lower alkyl radical and A is a lower alkylene radical.

3. As a composition of matter, a tetranitramine having the formula:



wherein R is a lower nitroalkyl radical and A is a lower alkylene radical.

4. As a composition of matter, 2,5,9,12-tetraaza-2,5,7,7,9,12-hexanitrotridecane having the structural formula:



5. As a composition of matter, 3,7,9,9,11,15-hexanitro-3,7,11,15-tetraazaheptadecane having the structural formula:



6. As a composition of matter, 2,2,4,7,9,9,11,14,16,16-decanitro-4,7,11,14-tetraazaheptadecane having the structural formula:



7. As a composition of matter, 2,2,4,7,9,9,11,15-octanitro-4,7,11,15-tetraazaheptadecane having the structural formula:



8. The method of preparing tetranitramines having the formula:



which comprises reacting a dinitramine having the formula:



with nitric acid; wherein R is a radical selected from the group consisting of hydrogen, lower alkyl and lower nitroalkyl radicals and A is a lower alkylene radical.

9. The method of claim 8 wherein the nitration reaction is conducted in the presence of sulfuric acid.

10. The method of preparing 2,5,9,12-tetraaza-2,5,7,7,9,12-hexanitrotridecane which comprises reacting 2,5,9,12-tetraaza-2,7,7,12-tetranitrotridecane with nitric acid.

11. The method of preparing 3,7,9,9,11,15-hexanitro-3,7,11,15-tetraazaheptadecane which comprises reacting 3,7,11,15-tetraazaheptadecane with nitric acid.

12. The method of preparing 2,2,4,7,9,9,11,14,16,16-decanitro-4,7,11,14-tetraazaheptadecane which comprises reacting 2,2,4,9,9,14,16,16-octanitro-4,7,11,14-tetraazaheptadecane with nitric acid.

13. The method of preparing tetranitramines having the formula:



which comprises reacting a dinitramine having the formula:



with nitric acid; wherein R is a lower alkyl radical and A is a lower alkylene radical.

14. The method of preparing tetranitramines having the formula:



which comprises reacting a dinitramine having the formula:



with nitric acid; wherein R is a lower nitroalkyl radical and A is a lower alkylene radical.

15. The method of claim 10 wherein the reaction is conducted in the presence of sulfuric acid.

16. The method of preparing 2,2,4,7,9,9,11,15-octanitro-4,7,11,15-tetraazaheptadecane which comprises reacting 2,2,4,9,9,15-hexanitro-4,7,11,15-tetraazaheptadecane with nitric acid.

55 No references cited.